

July 27, 1926.

1,594,038

E. E. BARTELS ET AL

HANDLING PRESSURE TAR

Filed Sept. 22, 1924



Inventors,  
Edward E. Bartels,  
Edward J. Shaefffer,  
By Dreyfus, Le Chatlier, Miles, Settig.

Patented July 27, 1926.

1,594,038

# UNITED STATES PATENT OFFICE.

EDWARD E. BARTELS AND EDWARD J. SHAEFFER, OF WHITING, INDIANA, ASSIGNEES  
TO STANDARD OIL COMPANY, OF WHITING, INDIANA, AND CHICAGO, ILLINOIS, A  
CORPORATION OF INDIANA.

## HANDLING PRESSURE TAR.

Application filed September 22, 1924. Serial No. 739,108.

The handling of pressure tar or the undistilled residuum from pressure cracking processes presents great difficulties, particularly in its redistillation either in continuous stills or coking stills, by reason of the large amounts of sediment which tends to deposit from the pressure tar. This sediment in coking processes, for example, frequently necessitates transferring entire batches of pressure tar undergoing distillation from one still to another by reason of excessive formation of coke and resulting hot bottoms in such stills.

The present invention relates to the handling of pressure tar in such a manner as to avoid such difficulties during the distillation of the tar, and to render useful the sedimentary matter deposited by the pressure tar. It will be fully understood from the following description, illustrated by the accompanying drawings, in which:

Figure 1 illustrates diagrammatically a system of tanks and connections employed in carrying out the present invention; and

Fig. 2 is a diagrammatic sectional view through one of the tanks of the series.

In carrying out the present invention, a plurality of tanks are employed for receiving the pressure tar from the pressure cracking system. For example, as shown diagrammatically in Fig. 1, three tanks of this character may be employed, designated respectively by the letters A, B and C. Pressure tar is supplied to a selected one of these tanks through the line 5, valved connections 6, 7 and 8 being provided from this line to the tanks A, B and C respectively. From the tanks the valved draw-off lines 9, 10 and 11 respectively lead to the intake line 12 of a pump 13, by which pressure tar drawn from a selected one of the tanks is forced through line 14 to the still (not shown). In operation, the tanks A, B and C are each in succession filled, permitted to settle and the pressure tar separated, and the separated clean pressure tar pumped to the pressure tar stills. Thus, while the tank A is being filled with pressure tar, that in the tank B is being allowed to settle, and that in the tank C is being drawn off by the pump 13. Rates of pumping are approximately adjusted so that, when tank C is empty, tank A is approximately filled. The pressure tar in tank A is permitted to settle, the

settled pressure tar in tank B is drawn off 55 and fresh pressure tar is pumped into tank C. The tanks are thus used in rotation.

As illustrated in Figure 2, which shows a diagrammatic section of tank A, upon settling, the pressure tar forms three fairly 60 distinct layers, an upper layer 15 of settled or clean pressure tar, a layer 16 of sediment or "B. S.", and a layer 17 of thicker or heavier sediment, designated "permanent B. S.". The pressure tar contains from 3 to 65 5% of materials which deposit in the two lower layers of sediment. These are allowed to accumulate until the upper surface of the upper layer of sediment 16 approaches a short distance, say 6 to 8 inches, of the 70 draw-off line for settled pressure tar, for example, the line 9 in the case of tank A. This line is elevated a considerable distance, say 4 to 16 inches above the bottom of the tank. The intermediate layer 16 of sediment is then drawn off through lower pipe 18, in the case of tank A, passing to the manifold suction line 19 of pump 20, by which the B. S. is pumped to the mixing tank 21. B. S. drawoff lines 22 and 23 are 80 provided for tanks B and C, respectively, corresponding to line 18 of tank A and connecting with the line 19.

After a quantity of the sediment or B. S. 16 has collected in any one of the tanks, it is 85 drawn out through the proper line, 18, 22 or 23, and forced by the pump 20 into the mixing tank 21. Into this tank a suitable quantity of heavy oil having a density of at least one, and preferably of from 1.03 to 90 1.07 is forced through line 24 into the tank 21. Oils suitable for this purpose are, for example, the road oils and fluxing oils obtained by steam reduction of pressure tar. Such oils have a density of 1.00 and higher 95 depending, upon the specific grade of oil. For example, a pressure tar residuum or road oil having a viscosity of 3 Engler at 212° F. and a specific gravity of about 1.04 at 60° has been found suitable for use. The 100 oils referred to range in viscosity from 1.5 to 6 Engler at 212° F. From 25% upwardly of the selected oil may be admixed with the pressure tar B. S., in general 50% being found suitable. Thorough admixture is effected, either by mechanical agitation or by air blast. The admixed oils are found not to deposit sediment on settling, and to be

excellently adapted for use as heavy fuel oils.

When the accumulation of permanent B. S. (the lowermost layer 17) becomes excessive, it is cleaned out by any suitable means, admixed with heavy oils of the character above described in the same manner as the intermediate sediment or B. S., and likewise used as fuel oil.

10 It is readily apparent that the sediment may be removed from the pressure tar by centrifuging or by other suitable means instead of by gravity settling.

We claim:

15 1. The method of handling pressure tar comprising settling the pressure tar, separately removing the settled tar and the sediment, and admixing the latter with a heavy oil having a specific gravity of at least 1 at 60° F.

20

2. The method of handling pressure tar comprising removing separable sediment from the pressure tar and admixing the sediment with a heavy oil having a specific gravity of at least 1 at 60° F.

25 3. The method of handling pressure tar comprising the steps of settling the pressure tar, separately removing the settled pressure tar and the sediment, and admixing the latter with a residuum from distillation of 30 pressure tar, said residuum having a specific gravity of at least 1.00 and a viscosity 1.5 to 6 Engler at 212° F.

4. The method of forming a fuel oil mixture which comprises admixing pressure tar 35 B. S. with a heavy oil having a density of at least 1.00.

EDWARD E. BARTELS.  
EDWARD J. SHAEFFER.